



US009016363B2

(12) **United States Patent**  
**Xu et al.**

(10) **Patent No.:** **US 9,016,363 B2**  
(45) **Date of Patent:** **\*Apr. 28, 2015**

(54) **DISINTEGRABLE METAL CONE, PROCESS OF MAKING, AND USE OF THE SAME**

(75) Inventors: **Zhiyue Xu**, Cypress, TX (US); **YingQing Xu**, Tomball, TX (US); **Gregory Lee Hern**, Porter, TX (US); **Bennett M. Richard**, Kingwood, TX (US)

(73) Assignee: **Baker Hughes Incorporated**, Houston, TX (US)

(\*) Notice: Subject to any disclaimer, the term of this patent is extended or adjusted under 35 U.S.C. 154(b) by 339 days.

This patent is subject to a terminal disclaimer.

(21) Appl. No.: **13/466,329**

(22) Filed: **May 8, 2012**

(65) **Prior Publication Data**

US 2013/0299185 A1 Nov. 14, 2013

(51) **Int. Cl.**

**E21B 33/1295** (2006.01)  
**E21B 33/12** (2006.01)  
**E21B 43/10** (2006.01)  
**B22F 3/24** (2006.01)  
**E21B 23/01** (2006.01)  
**E21B 33/134** (2006.01)

(Continued)

(52) **U.S. Cl.**

CPC ..... **E21B 43/106** (2013.01); **B22F 3/24** (2013.01); **E21B 33/12** (2013.01); **E21B 33/1295** (2013.01); **E21B 23/01** (2013.01); **E21B 33/134** (2013.01); **C22C 1/0408** (2013.01); **C22C 1/0416** (2013.01); **C22C 32/00** (2013.01); **B22F 2998/10** (2013.01)

(58) **Field of Classification Search**

USPC ..... 166/118, 135, 138, 192, 193, 216, 217,  
166/382

See application file for complete search history.

(56)

**References Cited**

U.S. PATENT DOCUMENTS

2,225,143 A \* 12/1940 Baker et al. ..... 166/119  
6,712,153 B2 3/2004 Turley et al.  
7,128,145 B2 10/2006 Mickey

(Continued)

OTHER PUBLICATIONS

Simulia Realistic Simulation News, [online]; [retrieved on Jan. 10, 2013]; retrieved from the internet [http://www.3ds.com/fileadmin/brands/SIMULIA/Customer\\_Stories/Baker\\_Hughes/Energy\\_BakerHughes\\_RSN\\_Feb11.pdf](http://www.3ds.com/fileadmin/brands/SIMULIA/Customer_Stories/Baker_Hughes/Energy_BakerHughes_RSN_Feb11.pdf), "Baker Hughes Refines Expandable Tubular Technology with Abaqus and Insight," Jan./Feb. 2011, 2p.

(Continued)

*Primary Examiner* — Kenneth L Thompson

(74) *Attorney, Agent, or Firm* — Cantor Colburn LLP

(57)

**ABSTRACT**

A frustoconical member includes a metal composite that has a cellular nanomatrix comprising a metallic nanomatrix material; a metal matrix disposed in the cellular nanomatrix; and a first frustoconical portion. A process of making the frustoconical member includes combining a metal matrix powder, a disintegration agent, and metal nanomatrix material to form a composition; compacting the composition to form a compacted composition; sintering the compacted composition; and pressing the sintered composition to form the frustoconical member having a tapered portion on an outer surface of the frustoconical member. The frustoconical member can be used by contacting a frustoconical portion of the frustoconical member to a tapered surface of an article; applying pressure to the frustoconical member; urging the frustoconical member in a direction relative to the article to expand a radial dimension of the article; and contacting the frustoconical member with a fluid to disintegrate the frustoconical member.

**30 Claims, 19 Drawing Sheets**



(51) **Int. Cl.**  
**C22C 1/04** (2006.01)  
**C22C 32/00** (2006.01)

(56) **References Cited**

## U.S. PATENT DOCUMENTS

|              |      |         |                      |         |
|--------------|------|---------|----------------------|---------|
| 7,168,494    | B2 * | 1/2007  | Starr et al. ....    | 166/379 |
| 7,210,533    | B2 * | 5/2007  | Starr et al. ....    | 166/376 |
| 2002/0139541 | A1   | 10/2002 | Sheffield et al.     |         |
| 2005/0098313 | A1   | 5/2005  | Atkins et al.        |         |
| 2006/0188602 | A1   | 8/2006  | Martin et al.        |         |
| 2008/0105438 | A1 * | 5/2008  | Jordan et al. ....   | 166/376 |
| 2008/0236842 | A1 * | 10/2008 | Bhavasar et al. .... | 166/381 |
| 2009/0065216 | A1   | 3/2009  | Frazier              |         |
| 2009/0139720 | A1   | 6/2009  | Frazier              |         |
| 2009/0211770 | A1   | 8/2009  | Nutley et al.        |         |
| 2010/0276159 | A1 * | 11/2010 | Mailand et al. ....  | 166/382 |
| 2011/0048743 | A1   | 3/2011  | Stafford et al.      |         |
| 2011/0132143 | A1   | 6/2011  | Xu et al.            |         |
| 2011/0132612 | A1   | 6/2011  | Agrawal et al.       |         |
| 2011/0132619 | A1   | 6/2011  | Agrawal et al.       |         |
| 2011/0132620 | A1   | 6/2011  | Agrawal et al.       |         |
| 2011/0259610 | A1 * | 10/2011 | Shkurti et al. ....  | 166/386 |

|              |      |         |                  |         |
|--------------|------|---------|------------------|---------|
| 2011/0314881 | A1   | 12/2011 | Hatcher et al.   |         |
| 2012/0205872 | A1   | 8/2012  | Reinhardt et al. |         |
| 2012/0234547 | A1   | 9/2012  | O'Malley et al.  |         |
| 2013/0048305 | A1 * | 2/2013  | Xu et al. ....   | 166/376 |
| 2013/0299192 | A1 * | 11/2013 | Xu et al. ....   | 166/382 |
| 2014/0262327 | A1 * | 9/2014  | Xu et al. ....   | 166/376 |

## OTHER PUBLICATIONS

Garry Garfield, "Formation Damage Control Utilizing Composite-Bridge-Plug Technology for Monobore, Multizone Stimulation Operations," SPE 70004, Copyright 2001, Society of Petroleum Engineers Inc., This paper was prepared for presentation at the SPE Permian Basin Oil and Gas Recovery Conference held in Midland, Texas, May 15-16, 2001, pp. 1-8.  
 International Search Report for related PCT Application No. PCT/US2013/035258, dated Jul. 4, 2013, pp. 1-4.  
 International Search Report for related PCT Application No. PCT/US2013/035261, dated Jul. 10, 2013, pp. 1-4.  
 International Search Report for related PCT Application No. PCT/US2013/035262, dated Jul. 1, 2013, pp. 1-4.  
 International Search Report for related PCT Application No. PCT/US2013/068062, dated Feb. 12, 2014, pp. 1-3.

\* cited by examiner



FIG. 1

200

FIG.2



FIG. 3

10, 30

FIG. 4



FIG.5A



FIG.5B



FIG. 6



FIG. 7A



FIG. 7B



FIG.8





FIG. 9B

514

FIG.10

700

FIG. 11



FIG. 12A



FIG. 12B



FIG. 12C



FIG. 13A



FIG. 13B





FIG. 15



FIG. 16



FIG. 17



FIG. 18A



FIG. 18B

## DISINTEGRABLE METAL CONE, PROCESS OF MAKING, AND USE OF THE SAME

### BACKGROUND

Downhole constructions including oil and natural gas wells, CO<sub>2</sub> sequestration boreholes, etc. often utilize borehole components or tools that, due to their function, are only required to have limited service lives that are considerably less than the service life of the well. After a component or tool service function is complete, it must be removed or disposed of in order to recover the original size of the fluid pathway for use, including hydrocarbon production, CO<sub>2</sub> capture or sequestration, etc. Disposal of components or tools can be accomplished by milling or drilling the component or tool out of the borehole, which is generally a time consuming and expensive operation. The industry is always receptive to new systems, materials, and methods that eliminate removal of a component or tool from a borehole without such milling and drilling operations.

### BRIEF DESCRIPTION

Disclosed herein is a frustoconical member comprising: a metal composite including: a cellular nanomatrix comprising a metallic nanomatrix material; a metal matrix disposed in the cellular nanomatrix; and a first frustoconical portion.

Also disclosed is a process of making a frustoconical member, the process comprising: combining a metal matrix powder, a disintegration agent, and metal nanomatrix material to form a composition; compacting the composition to form a compacted composition; sintering the compacted composition; and pressing the sintered composition to form the frustoconical member having a tapered portion on an outer surface of the frustoconical member.

Further disclosed is a method of using a frustoconical member, the method comprising: contacting a frustoconical portion of the frustoconical member to a tapered surface of an article; applying pressure to the frustoconical member; urging the frustoconical member in a direction relative to the article to expand a radial dimension of the article; and contacting the frustoconical member with a fluid to disintegrate the frustoconical member.

### BRIEF DESCRIPTION OF THE DRAWINGS

The following descriptions should not be considered limiting in any way. With reference to the accompanying drawings, like elements are numbered alike:

FIG. 1 depicts a cross sectional view of a disintegrable tubular anchoring system;

FIG. 2 depicts a cross sectional view of a disintegrable metal composite;

FIG. 3 is a photomicrograph of an exemplary embodiment of a disintegrable metal composite as disclosed herein;

FIG. 4 depicts a cross sectional view of a composition used to make the disintegrable metal composite shown in FIG. 2;

FIG. 5A is a photomicrograph of a pure metal without a cellular nanomatrix;

FIG. 5B is a photomicrograph of a disintegrable metal composite with a metal matrix and cellular nanomatrix;

FIG. 6 is a graph of mass loss versus time for various disintegrable metal composites that include a cellular nanomatrix indicating selectively tailorable disintegration rates;

FIG. 7A is an electron photomicrograph of a fracture surface of a compact formed from a pure Mg powder;

FIG. 7B is an electron photomicrograph of a fracture surface of an exemplary embodiment of a disintegrable metal composite with a cellular nanomatrix as described herein;

FIG. 8 is a graph of the compressive strength of a metal composite with a cellular nanomatrix versus weight percentage of a constituent (Al<sub>2</sub>O<sub>3</sub>) of the cellular nanomatrix;

FIG. 9A depicts a cross sectional view of an embodiment of a disintegrable tubular anchoring system in a borehole;

FIG. 9B depicts a cross sectional view of the system of FIG. 9A in a set position;

FIG. 10 depicts a cross sectional view of a disintegrable frustoconical member;

FIG. 11 depicts a cross sectional view of a disintegrable bottom sub;

FIGS. 12A, 12B, and 12C respectively depict a perspective view, cross sectional view, and a top view of a disintegrable sleeve;

FIGS. 13A and 13B respectively depict a perspective view and cross sectional view of a disintegrable seal;

FIG. 14 depicts a cross sectional view of another embodiment of a disintegrable tubular anchoring system;

FIG. 15 depicts a cross sectional view of the disintegrable tubular anchoring system of FIG. 14 in a set position;

FIG. 16 depicts a cross sectional view of another embodiment of a disintegrable tubular anchoring system;

FIG. 17 depicts a cross sectional view of another embodiment of a disintegrable seal with an elastomer backup ring in a disintegrable tubular anchoring system; and

FIGS. 18A and 18B respectively depict a cross sectional and perspective views of another embodiment of a disintegrable seal.

### DETAILED DESCRIPTION

35 A detailed description of one or more embodiments of the disclosed apparatus and method are presented herein by way of exemplification and not limitation with reference to the Figures.

The inventors have discovered that a high strength, high 40 ductility yet fully disintegrable tubular anchoring system can be made from materials that selectively and controllably disintegrate in response to contact with certain downhole fluids or in response to changed conditions. Such a disintegrable system includes components that are selectively corrodible

45 and have selectively tailorable disintegration rates and selectively tailor able material properties. Additionally, the disintegrable system has components that have varying compression and tensile strengths and that include a seal (to form, e.g., a conformable metal-to-metal seal), cone, deformable sleeve (or slips), and bottom sub. As used herein, "disintegrable" refers to a material or component that is consumable, corrodible, degradable, dissolvable, weakenable, or otherwise removable. It is to be understood that use herein of the term "disintegrate," or any of its forms (e.g., "disintegration"), 50 incorporates the stated meaning.

An embodiment of a disintegrable tubular anchoring system is shown in FIG. 1. The disintegrable tubular anchoring system 110 includes a seal 112, frustoconical member 114, a sleeve 116 (shown herein as a slip ring), and a bottom sub 118. 55 The system 110 is configured such that longitudinal movement of the frustoconical member 114 relative to the sleeve 116 and relative to the seal 112 causes the sleeve 116 and seal 112 respectively to be radially altered. Although in this embodiment the radial alterations are in radially outward directions, in alternate embodiments the radial alterations could be in other directions such as radially inward. Additionally, a longitudinal dimension D1 and thickness T1 of a wall

portion of the seal 112 can be altered upon application of a compressive force thereto. The seal 112, frustoconical member 114, sleeve 116, and bottom sub 118 (i.e., components of the system 110) are disintegrable and contain a metal composite. The metal composite includes a metal matrix disposed in a cellular nanomatrix and a disintegration agent.

In an embodiment, the disintegration agent is disposed in the metal matrix. In another embodiment, the disintegration agent is disposed external to the metal matrix. In yet another embodiment, the disintegration agent is disposed in the metal matrix as well as external to the metal matrix. The metal composite also includes the cellular nanomatrix that comprises a metallic nanomatrix material. The disintegration agent can be disposed in the cellular nanomatrix among the metallic nanomatrix material. An exemplary metal composite and method used to make the metal composite are disclosed in U.S. patent application Ser. Nos. 12/633,682, 12/633,688, 13/220,832, 13/220,822, and 13/358,307, the disclosure of each of which patent application is incorporated herein by reference in its entirety.

The metal composite is, for example, a powder compact as shown in FIG. 2. The metal composite 200 includes a cellular nanomatrix 216 comprising a nanomatrix material 220 and a metal matrix 214 (e.g., a plurality of dispersed particles) comprising a particle core material 218 dispersed in the cellular nanomatrix 216. The particle core material 218 comprises a nanostructured material. Such a metal composite having the cellular nanomatrix with metal matrix disposed therein is referred to as controlled electrolytic material.

With reference to FIGS. 2 and 4, metal matrix 214 can include any suitable metallic particle core material 218 that includes nanostructure as described herein. In an exemplary embodiment, the metal matrix 214 is formed from particle cores 14 (FIG. 4) and can include an element such as aluminum, iron, magnesium, manganese, zinc, or a combination thereof, as the nanostructured particle core material 218. More particularly, in an exemplary embodiment, the metal matrix 214 and particle core material 218 can include various Al or Mg alloys as the nanostructured particle core material 218, including various precipitation hardenable alloys Al or Mg alloys. In some embodiments, the particle core material 218 includes magnesium and aluminum where the aluminum is present in an amount of about 1 weight percent (wt %) to about 15 wt %, specifically about 1 wt % to about 10 wt %, and more specifically about 1 wt % to about 5 wt %, based on the weight of the metal matrix, the balance of the weight being magnesium.

In an additional embodiment, precipitation hardenable Al or Mg alloys are particularly useful because they can strengthen the metal matrix 214 through both nanostructuring and precipitation hardening through the incorporation of particle precipitates as described herein. The metal matrix 214 and particle core material 218 also can include a rare earth element, or a combination of rare earth elements. Exemplary rare earth elements include Sc, Y, La, Ce, Pr, Nd, or Er. A combination comprising at least one of the foregoing rare earth elements can be used. Where present, the rare earth element can be present in an amount of about 5 wt % or less, and specifically about 2 wt % or less, based on the weight of the metal composite.

The metal matrix 214 and particle core material 218 also can include a nanostructured material 215. In an exemplary embodiment, the nanostructured material 215 is a material having a grain size (e.g., a subgrain or crystallite size) that is less than about 200 nanometers (nm), specifically about 10 nm to about 200 nm, and more specifically an average grain size less than about 100 nm. The nanostructure of the metal

matrix 214 can include high angle boundaries 227, which are usually used to define the grain size, or low angle boundaries 229 that may occur as substructure within a particular grain, which are sometimes used to define a crystallite size, or a combination thereof. It will be appreciated that the nanocellular matrix 216 and grain structure (nanostructured material 215 including grain boundaries 227 and 229) of the metal matrix 214 are distinct features of the metal composite 200. Particularly, nanocellular matrix 216 is not part of a crystalline or amorphous portion of the metal matrix 214.

The disintegration agent is included in the metal composite 200 to control the disintegration rate of the metal composite 200. The disintegration agent can be disposed in the metal matrix 214, the cellular nanomatrix 216, or a combination thereof. According to an embodiment, the disintegration agent includes a metal, fatty acid, ceramic particle, or a combination comprising at least one of the foregoing, the disintegration agent being disposed among the controlled electrolytic material to change the disintegration rate of the controlled electrolytic material. In one embodiment, the disintegration agent is disposed in the cellular nanomatrix external to the metal matrix. In a non-limiting embodiment, the disintegration agent increases the disintegration rate of the metal composite 200. In another embodiment, the disintegration agent decreases the disintegration rate of the metal composite 200. The disintegration agent can be a metal including cobalt, copper, iron, nickel, tungsten, zinc, or a combination comprising at least one of the foregoing. In a further embodiment, the disintegration agent is the fatty acid, e.g., fatty acids having 6 to 40 carbon atoms. Exemplary fatty acids include oleic acid, stearic acid, lauric acid, hydroxystearic acid, behenic acid, arachidonic acid, linoleic acid, linolenic acid, ricinoleic acid, palmitic acid, montanic acid, or a combination comprising at least one of the foregoing. In yet another embodiment, the disintegration agent is ceramic particles such as boron nitride, tungsten carbide, tantalum carbide, titanium carbide, niobium carbide, zirconium carbide, boron carbide, hafnium carbide, silicon carbide, niobium boron carbide, aluminum nitride, titanium nitride, zirconium nitride, tantalum nitride, or a combination comprising at least one of the foregoing. Additionally, the ceramic particle can be one of the ceramic materials discussed below with regard to the strengthening agent. Such ceramic particles have a size of 5  $\mu\text{m}$  or less, specifically 2  $\mu\text{m}$  or less, and more specifically 1  $\mu\text{m}$  or less. The disintegration agent can be present in an amount effective to cause disintegration of the metal composite 200 at a desired disintegration rate, specifically about 0.25 wt % to about 15 wt %, specifically about 0.25 wt % to about 10 wt %, specifically about 0.25 wt % to about 1 wt %, based on the weight of the metal composite.

In an exemplary embodiment, the cellular nanomatrix 216 includes aluminum, cobalt, copper, iron, magnesium, nickel, silicon, tungsten, zinc, an oxide thereof, a nitride thereof, a carbide thereof, an intermetallic compound thereof, a cermet thereof, or a combination comprising at least one of the foregoing. The metal matrix can be present in an amount from about 50 wt % to about 95 wt %, specifically about 60 wt % to about 95 wt %, and more specifically about 70 wt % to about 95 wt %, based on the weight of the seal. Further, the amount of the metal nanomatrix material is about 10 wt % to about 50 wt %, specifically about 20 wt % to about 50 wt %, and more specifically about 30 wt % to about 50 wt %, based on the weight of the seal.

In another embodiment, the metal composite includes a second particle. As illustrated generally in FIGS. 2 and 4, the metal composite 200 can be formed using a coated metallic powder 10 and an additional or second powder 30, i.e., both

powders **10** and **30** can have substantially the same particulate structure without having identical chemical compounds. The use of an additional powder **30** provides a metal composite **200** that also includes a plurality of dispersed second particles **234**, as described herein, that are dispersed within the cellular nanomatrix **216** and are also dispersed with respect to the metal matrix **214**. Thus, the dispersed second particles **234** are derived from second powder particles **32** disposed in the powder **10**, **30**. In an exemplary embodiment, the dispersed second particles **234** include Ni, Fe, Cu, Co, W, Al, Zn, Mn, Si, an oxide thereof, nitride thereof, carbide thereof, intermetallic compound thereof, cermet thereof, or a combination comprising at least one of the foregoing.

Referring again to FIG. 2, the metal matrix **214** and particle core material **218** also can include an additive particle **222**. The additive particle **222** provides a dispersion strengthening mechanism to the metal matrix **214** and provides an obstacle to, or serves to restrict, the movement of dislocations within individual particles of the metal matrix **214**. Additionally, the additive particle **222** can be disposed in the cellular nanomatrix **216** to strengthen the metal composite **200**. The additive particle **222** can have any suitable size and, in an exemplary embodiment, can have an average particle size of about 10 nm to about 1 micron, and specifically about 50 nm to about 200 nm. Here, size refers to the largest linear dimension of the additive particle. The additive particle **222** can include any suitable form of particle, including an embedded particle **224**, a precipitate particle **226**, or a dispersoid particle **228**. Embedded particle **224** can include any suitable embedded particle, including various hard particles. The embedded particle can include various metal, carbon, metal oxide, metal nitride, metal carbide, intermetallic compound, cermet particle, or a combination thereof. In an exemplary embodiment, hard particles can include Ni, Fe, Cu, Co, W, Al, Zn, Mn, Si, an oxide thereof, nitride thereof, carbide thereof, intermetallic compound thereof, cermet thereof, or a combination comprising at least one of the foregoing. The additive particle can be present in an amount of about 0.5 wt % to about 25 wt %, specifically about 0.5 wt % to about 20 wt %, and more specifically about 0.5 wt % to about 10 wt %, based on the weight of the metal composite.

In metal composite **200**, the metal matrix **214** dispersed throughout the cellular nanomatrix **216** can have an equiaxed structure in a substantially continuous cellular nanomatrix **216** or can be substantially elongated along an axis so that individual particles of the metal matrix **214** are oblately or prolately shaped, for example. In the case where the metal matrix **214** has substantially elongated particles, the metal matrix **214** and the cellular nanomatrix **216** may be continuous or discontinuous. The size of the particles that make up the metal matrix **214** can be from about 50 nm to about 800  $\mu\text{m}$ , specifically about 500 nm to about 600  $\mu\text{m}$ , and more specifically about 1  $\mu\text{m}$  to about 500  $\mu\text{m}$ . The particle size of can be monodisperse or polydisperse, and the particle size distribution can be unimodal or bimodal. Size here refers to the largest linear dimension of a particle.

Referring to FIG. 3 a photomicrograph of an exemplary embodiment of a metal composite is shown. The metal composite **300** has a metal matrix **214** that includes particles having a particle core material **218**. Additionally, each particle of the metal matrix **214** is disposed in a cellular nanomatrix **216**. Here, the cellular nanomatrix **216** is shown as a white network that substantially surrounds the component particles of the metal matrix **214**.

According to an embodiment, the metal composite is formed from a combination of, for example, powder constituents. As illustrated in FIG. 4, a powder **10** includes powder

particles **12** that have a particle core **14** with a core material **18** and metallic coating layer **16** with coating material **20**. These powder constituents can be selected and configured for compaction and sintering to provide the metal composite **200** that is lightweight (i.e., having a relatively low density), high-strength, and selectively and controllably removable, e.g., by disintegration, from a borehole in response to a change in a borehole property, including being selectively and controllably disintegrable (e.g., by having a selectively tailorable disintegration rate curve) in an appropriate borehole fluid, including various borehole fluids as disclosed herein.

The nanostructure can be formed in the particle core **14** used to form metal matrix **214** by any suitable method, including a deformation-induced nanostructure such as can be provided by ball milling a powder to provide particle cores **14**, and more particularly by cryomilling (e.g., ball milling in ball milling media at a cryogenic temperature or in a cryogenic fluid, such as liquid nitrogen) a powder to provide the particle cores **14** used to form the metal matrix **214**. The particle cores **14** may be formed as a nanostructured material **215** by any suitable method, such as, for example, by milling or cryomilling of prealloyed powder particles of the materials described herein. The particle cores **14** may also be formed by mechanical alloying of pure metal powders of the desired amounts of the various alloy constituents. Mechanical alloying involves ball milling, including cryomilling, of these powder constituents to mechanically enfold and intermix the constituents and form particle cores **14**. In addition to the creation of nanostructure as described above, ball milling, including cryomilling, can contribute to solid solution strengthening of the particle core **14** and core material **18**, which in turn can contribute to solid solution strengthening of the metal matrix **214** and particle core material **218**. The solid solution strengthening can result from the ability to mechanically intermix a higher concentration of interstitial or substitutional solute atoms in the solid solution than is possible in accordance with the particular alloy constituent phase equilibria, thereby providing an obstacle to, or serving to restrict, the movement of dislocations within the particle, which in turn provides a strengthening mechanism in the particle core **14** and the metal matrix **214**. The particle core **14** can also be formed with a nanostructure (grain boundaries **227**, **229**) by methods including inert gas condensation, chemical vapor condensation, pulse electron deposition, plasma synthesis, crystallization of amorphous solids, electrodeposition, and severe plastic deformation, for example. The nanostructure also can include a high dislocation density, such as, for example, a dislocation density between about  $10^{17} \text{ m}^{-2}$  and about  $10^{18} \text{ m}^{-2}$ , which can be two to three orders of magnitude higher than similar alloy materials deformed by traditional methods, such as cold rolling.

The substantially-continuous cellular nanomatrix **216** (see FIG. 3) and nanomatrix material **220** formed from metallic coating layers **16** by the compaction and sintering of the plurality of metallic coating layers **16** with the plurality of powder particles **12**, such as by cold isostatic pressing (CIP), hot isostatic pressing (HIP), or dynamic forging. The chemical composition of nanomatrix material **220** may be different than that of coating material **20** due to diffusion effects associated with the sintering. The metal composite **200** also includes a plurality of particles that make up the metal matrix **214** that comprises the particle core material **218**. The metal matrix **214** and particle core material **218** correspond to and are formed from the plurality of particle cores **14** and core material **18** of the plurality of powder particles **12** as the metallic coating layers **16** are sintered together to form the cellular nanomatrix **216**. The chemical composition of par-

ticle core material 218 may also be different than that of core material 18 due to diffusion effects associated with sintering.

As used herein, the term cellular nanomatrix 216 does not connote the major constituent of the powder compact, but rather refers to the minority constituent or constituents, whether by weight or by volume. This is distinguished from most matrix composite materials where the matrix comprises the majority constituent by weight or volume. The use of the term substantially continuous, cellular nanomatrix is intended to describe the extensive, regular, continuous and interconnected nature of the distribution of nanomatrix material 220 within the metal composite 200. As used herein, "substantially continuous" describes the extension of the nanomatrix material 220 throughout the metal composite 200 such that it extends between and envelopes substantially all of the metal matrix 214. Substantially continuous is used to indicate that complete continuity and regular order of the cellular nanomatrix 220 around individual particles of the metal matrix 214 are not required. For example, defects in the coating layer 16 over particle core 14 on some powder particles 12 may cause bridging of the particle cores 14 during sintering of the metal composite 200, thereby causing localized discontinuities to result within the cellular nanomatrix 216, even though in the other portions of the powder compact the cellular nanomatrix 216 is substantially continuous and exhibits the structure described herein. In contrast, in the case of substantially elongated particles of the metal matrix 214 (i.e., non-equiaxed shapes), such as those formed by extrusion, "substantially discontinuous" is used to indicate that incomplete continuity and disruption (e.g., cracking or separation) of the nanomatrix around each particle of the metal matrix 214, such as may occur in a predetermined extrusion direction. As used herein, "cellular" is used to indicate that the nanomatrix defines a network of generally repeating, interconnected, compartments or cells of nanomatrix material 220 that encompass and also interconnect the metal matrix 214. As used herein, "nanomatrix" is used to describe the size or scale of the matrix, particularly the thickness of the matrix between adjacent particles of the metal matrix 214. The metallic coating layers that are sintered together to form the nanomatrix are themselves nanoscale thickness coating layers. Since the cellular nanomatrix 216 at most locations, other than the intersection of more than two particles of the metal matrix 214, generally comprises the interdiffusion and bonding of two coating layers 16 from adjacent powder particles 12 having nanoscale thicknesses, the cellular nanomatrix 216 formed also has a nanoscale thickness (e.g., approximately two times the coating layer thickness as described herein) and is thus described as a nanomatrix. Further, the use of the term metal matrix 214 does not connote the minor constituent of metal composite 200, but rather refers to the majority constituent or constituents, whether by weight or by volume. The use of the term metal matrix is intended to convey the discontinuous and discrete distribution of particle core material 218 within metal composite 200.

Embedded particle 224 can be embedded by any suitable method, including, for example, by ball milling or cryomilling hard particles together with the particle core material 18. A precipitate particle 226 can include any particle that can be precipitated within the metal matrix 214, including precipitate particles 226 consistent with the phase equilibria of constituents of the materials, particularly metal alloys, of interest and their relative amounts (e.g., a precipitation hardenable alloy), and including those that can be precipitated due to non-equilibrium conditions, such as may occur when an alloy constituent that has been forced into a solid solution of the alloy in an amount above its phase equilibrium limit, as is

known to occur during mechanical alloying, is heated sufficiently to activate diffusion mechanisms that enable precipitation. Dispersoid particles 228 can include nanoscale particles or clusters of elements resulting from the manufacture of the particle cores 14, such as those associated with ball milling, including constituents of the milling media (e.g., balls) or the milling fluid (e.g., liquid nitrogen) or the surfaces of the particle cores 14 themselves (e.g., metallic oxides or nitrides). Dispersoid particles 228 can include an element such as, for example, Fe, Ni, Cr, Mn, N, O, C, H, and the like. The additive particles 222 can be disposed anywhere in conjunction with particle cores 14 and the metal matrix 214. In an exemplary embodiment, additive particles 222 can be disposed within or on the surface of metal matrix 214 as illustrated in FIG. 2. In another exemplary embodiment, a plurality of additive particles 222 are disposed on the surface of the metal matrix 214 and also can be disposed in the cellular nanomatrix 216 as illustrated in FIG. 2.

Similarly, dispersed second particles 234 may be formed from coated or uncoated second powder particles 32 such as by dispersing the second powder particles 32 with the powder particles 12. In an exemplary embodiment, coated second powder particles 32 may be coated with a coating layer 36 that is the same as coating layer 16 of powder particles 12, such that coating layers 36 also contribute to the nanomatrix 216. In another exemplary embodiment, the second powder particles 232 may be uncoated such that dispersed second particles 234 are embedded within nanomatrix 216. The powder 10 and additional powder 30 may be mixed to form a homogeneous dispersion of dispersed particles 214 and dispersed second particles 234 or to form a non-homogeneous dispersion of these particles. The dispersed second particles 234 may be formed from any suitable additional powder 30 that is different from powder 10, either due to a compositional difference in the particle core 34, or coating layer 36, or both of them, and may include any of the materials disclosed herein for use as second powder 30 that are different from the powder 10 that is selected to form powder compact 200.

In an embodiment, the metal composite optionally includes a strengthening agent. The strengthening agent increases the material strength of the metal composite. Exemplary strengthening agents include a ceramic, polymer, metal, nanoparticles, cermet, and the like. In particular, the strengthening agent can be silica, glass fiber, carbon fiber, carbon black, carbon nanotubes, oxides, carbides, nitrides, silicides, borides, phosphides, sulfides, cobalt, nickel, iron, tungsten, molybdenum, tantalum, titanium, chromium, niobium, boron, zirconium, vanadium, silicon, palladium, hafnium, aluminum, copper, or a combination comprising at least one of the foregoing. According to an embodiment, a ceramic and metal is combined to form a cermet, e.g., tungsten carbide, cobalt nitride, and the like. Exemplary strengthening agents particularly include magnesia, mullite, thoria, beryllia, urania, spinels, zirconium oxide, bismuth oxide, aluminum oxide, magnesium oxide, silica, barium titanate, cordierite, boron nitride, tungsten carbide, tantalum carbide, titanium carbide, niobium carbide, zirconium carbide, boron carbide, hafnium carbide, silicon carbide, niobium boron carbide, aluminum nitride, titanium nitride, zirconium nitride, tantalum nitride, hafnium nitride, niobium nitride, boron nitride, silicon nitride, titanium boride, chromium boride, zirconium boride, tantalum boride, molybdenum boride, tungsten boride, cerium sulfide, titanium sulfide, magnesium sulfide, zirconium sulfide, or a combination comprising at least one of the foregoing.

In one embodiment, the strengthening agent is a particle with size of about 100 microns or less, specifically about 10

microns or less, and more specifically 500 nm or less. In another embodiment, a fibrous strengthening agent can be combined with a particulate strengthening agent. It is believed that incorporation of the strengthening agent can increase the strength and fracture toughness of the metal composite. Without wishing to be bound by theory, finer (i.e., smaller) sized particles can produce a stronger metal composite as compared with larger sized particles. Moreover, the shape of strengthening agent can vary and includes fiber, sphere, rod, tube, and the like. The strengthening agent can be present in an amount of 0.01 weight percent (wt %) to 20 wt %, specifically 0.01 wt % to 10 wt %, and more specifically 0.01 wt % to 5 wt %.

In a process for preparing a component of a disintegrable anchoring system (e.g., a seal, frustoconical member, sleeve, bottom sub, and the like) containing a metal composite, the process includes combining a metal matrix powder, disintegration agent, metal nanomatrix material, and optionally a strengthening agent to form a composition; compacting the composition to form a compacted composition; sintering the compacted composition; and pressing the sintered composition to form the component of the disintegrable system. The members of the composition can be mixed, milled, blended, and the like to form the powder 10 as shown in FIG. 4 for example. It should be appreciated that the metal nanomatrix material is a coating material disposed on the metal matrix powder that, when compacted and sintered, forms the cellular nanomatrix. A compact can be formed by pressing (i.e., compacting) the composition at a pressure to form a green compact. The green compact can be subsequently pressed under a pressure of about 15,000 psi to about 100,000 psi, specifically about 20,000 psi to about 80,000 psi, and more specifically about 30,000 psi to about 70,000 psi, at a temperature of about 250° C. to about 600° C., and specifically about 300° C. to about 450° C., to form the powder compact. Pressing to form the powder compact can include compression in a mold. The powder compact can be further machined to shape the powder compact to a useful shape. Alternatively, the powder compact can be pressed into the useful shape. Machining can include cutting, sawing, ablating, milling, facing, lathing, boring, and the like using, for example, a mill, table saw, lathe, router, electric discharge machine, and the like.

The metal matrix 200 can have any desired shape or size, including that of a cylindrical billet, bar, sheet, toroid, or other form that may be machined, formed or otherwise used to form useful articles of manufacture, including various wellbore tools and components. Pressing is used to form a component of the disintegrable anchoring system (e.g., seal, frustoconical member, sleeve, bottom sub, and the like) from the sintering and pressing processes used to form the metal composite 200 by deforming the powder particles 12, including particle cores 14 and coating layers 16, to provide the full density and desired macroscopic shape and size of the metal composite 200 as well as its microstructure. The morphology (e.g., equiaxed or substantially elongated) of the individual particles of the metal matrix 214 and cellular nanomatrix 216 of particle layers results from sintering and deformation of the powder particles 12 as they are compacted and interdiffuse and deform to fill the interparticle spaces of the metal matrix 214 (FIG. 2). The sintering temperatures and pressures can be selected to ensure that the density of the metal composite 200 achieves substantially full theoretical density.

The metal composite has beneficial properties for use in, for example a downhole environment. In an embodiment, a component of the disintegrable anchoring system made of the metal composite has an initial shape that can be run downhole and, in the case of the seal and sleeve, can be subsequently

deformed under pressure. The metal composite is strong and ductile with a percent elongation of about 0.1% to about 75%, specifically about 0.1% to about 50%, and more specifically about 0.1% to about 25%, based on the original size of the 5 component of the disintegrable anchoring system. The metal composite has a yield strength of about 15 kilopounds per square inch (ksi) to about 50 ksi, and specifically about 15 ksi to about 45 ksi. The compressive strength of the metal composite is from about 30 ksi to about 100 ksi, and specifically 10 about 40 ksi to about 80 ksi. The components of the disintegrable anchoring system can have the same or different material properties, such as percent elongation, compressive strength, tensile strength, and the like.

Unlike elastomeric materials, the components of the disintegrable anchoring system herein that include the metal composite have a temperature rating up to about 1200° F., specifically up to about 1000° F., and more specifically about 800° F. The disintegrable anchoring system is temporary in that the 15 system is selectively and tailorably disintegrable in response to contact with a downhole fluid or change in condition (e.g., pH, temperature, pressure, time, and the like). Moreover, the components of the disintegrable anchoring system can have the same or different disintegration rates or reactivities with the downhole fluid. Exemplary downhole fluids include 20 brine, mineral acid, organic acid, or a combination comprising at least one of the foregoing. The brine can be, for example, seawater, produced water, completion brine, or a combination thereof. The properties of the brine can depend on the identity and components of the brine. Seawater, as an 25 example, contains numerous constituents such as sulfate, bromine, and trace metals, beyond typical halide-containing salts. On the other hand, produced water can be water extracted from a production reservoir (e.g., hydrocarbon reservoir), produced from the ground. Produced water is also 30 referred to as reservoir brine and often contains many components such as barium, strontium, and heavy metals. In addition to the naturally occurring brines (seawater and produced water), completion brine can be synthesized from fresh water by addition of various salts such as KCl, NaCl, ZnCl<sub>2</sub>, 35 MgCl<sub>2</sub>, or CaCl<sub>2</sub> to increase the density of the brine, such as 10.6 pounds per gallon of CaCl<sub>2</sub> brine. Completion brines 40 typically provide a hydrostatic pressure optimized to counter the reservoir pressures downhole. The above brines can be modified to include an additional salt. In an embodiment, the additional salt included in the brine is NaCl, KCl, NaBr, MgCl<sub>2</sub>, CaCl<sub>2</sub>, CaBr<sub>2</sub>, ZnBr<sub>2</sub>, NH<sub>4</sub>Cl, sodium formate, 45 cesium formate, and the like. The salt can be present in the brine in an amount from about 0.5 wt. % to about 50 wt. %, specifically about 1 wt. % to about 40 wt. %, and more 50 specifically about 1 wt. % to about 25 wt. %, based on the weight of the composition.

In another embodiment, the downhole fluid is a mineral acid that can include hydrochloric acid, nitric acid, phosphoric acid, sulfuric acid, boric acid, hydrofluoric acid, hydrobromic acid, perchloric acid, or a combination comprising at 55 least one of the foregoing. In yet another embodiment, the downhole fluid is an organic acid that can include a carboxylic acid, sulfonic acid, or a combination comprising at least one of the foregoing. Exemplary carboxylic acids include formic acid, acetic acid, chloroacetic acid, dichloroacetic acid, trichloroacetic acid, trifluoroacetic acid, propionic acid, butyric acid, oxalic acid, benzoic acid, phthalic acid (including ortho-, meta- and para-isomers), and the like. Exemplary sulfonic acids include alkyl sulfonic acid or aryl sulfonic acid. 60 Alkyl sulfonic acids include, e.g., methane sulfonic acid. Aryl sulfonic acids include, e.g., benzene sulfonic acid or toluene sulfonic acid. In one embodiment, the alkyl group may be

branched or unbranched and may contain from one to about 20 carbon atoms and can be substituted or unsubstituted. The aryl group can be alkyl-substituted, i.e., may be an alkylaryl group, or may be attached to the sulfonic acid moiety via an alkylene group (i.e., an arylalkyl group). In an embodiment, the aryl group may be substituted with a heteroatom. The aryl group can have from about 3 carbon atoms to about 20 carbon atoms and include a polycyclic ring structure.

The disintegration rate (also referred to as dissolution rate) of the metal composite is about 1 milligram per square centimeter per hour (mg/cm<sup>2</sup>/hr) to about 10,000 mg/cm<sup>2</sup>/hr, specifically about 25 mg/cm<sup>2</sup>/hr to about 1000 mg/cm<sup>2</sup>/hr, and more specifically about 50 mg/cm<sup>2</sup>/hr to about 500 mg/cm<sup>2</sup>/hr. The disintegration rate is variable upon the composition and processing conditions used to form the metal composite herein.

Without wishing to be bound by theory, the unexpectedly high disintegration rate of the metal composite herein is due to the microstructure provided by the metal matrix and cellular nanomatrix. As discussed above, such microstructure is provided by using powder metallurgical processing (e.g., compaction and sintering) of coated powders, wherein the coating produces the nanocellular matrix and the powder particles produce the particle core material of the metal matrix. It is believed that the intimate proximity of the cellular nanomatrix to the particle core material of the metal matrix in the metal composite produces galvanic sites for rapid and tailorably disintegration of the metal matrix. Such electrolytic sites are missing in single metals and alloys that lack a cellular nanomatrix. For illustration, FIG. 5A shows a compact 50 formed from magnesium powder. Although the compact 50 exhibits particles 52 surrounded by particle boundaries 54, the particle boundaries constitute physical boundaries between substantially identical material (particles 52). However, FIG. 5B shows an exemplary embodiment of a composite metal 56 (a powder compact) that includes a metal matrix 58 having particle core material 60 disposed in a cellular nanomatrix 62. The composite metal 56 was formed from aluminum oxide coated magnesium particles where, under powder metallurgical processing, the aluminum oxide coating produces the cellular nanomatrix 62, and the magnesium produces the metal matrix 58 having particle core material 60 (of magnesium). Cellular nanomatrix 62 is not just a physical boundary as the particle boundary 54 in FIG. 5A but is also a chemical boundary interposed between neighboring particle core materials 60 of the metal matrix 58. Whereas the particles 52 and particle boundary 54 in compact 50 (FIG. 5A) do not have galvanic sites, metal matrix 58 having particle core material 60 establish a plurality of galvanic sites in conjunction with the cellular nanomatrix 62. The reactivity of the galvanic sites depend on the compounds used in the metal matrix 58 and the cellular nanomatrix 62 as is an outcome of the processing conditions used to the metal matrix and cellular nanomatrix microstructure of the metal composite.

Moreover, the microstructure of the metal composites herein is controllable by selection of powder metallurgical processing conditions and chemical materials used in the powders and coatings. Therefore, the disintegration rate is selectively tailorable as illustrated for metal composites of various compositions in FIG. 6, which shows a graph of mass loss versus time for various metal composites that include a cellular nanomatrix. Specifically, FIG. 6 displays disintegration rate curves for four different metal composites (metal composite A 80, metal composite B 82 metal composite C 84, and metal composite D 86). The slope of each segment of each curve (separated by the black dots in FIG. 6) provides the disintegration rate for particular segments of the curve. Metal

composite A 80 has two distinct disintegration rates (802, 806). Metal composite B 82 has three distinct disintegration rates (808, 812, 816). Metal composite C 84 has two distinct disintegration rates (818, 822), and metal composite D 86 has four distinct disintegration rates (824, 828, 832, and 836). At a time represented by points 804, 810, 814, 820, 826, 830, and 834, the rate of the disintegration of the metal composite (80, 82, 84, 86) changes due to a changed condition (e.g., pH, temperature, time, pressure as discussed above). The rate may increase (e.g., going from rate 818 to rate 822) or decrease (e.g., going from rate 802 to 806) along the same disintegration curve. Moreover, a disintegration rate curve can have more than two rates, more than three rates, more than four rates, etc. based on the microstructure and components of the metallic composite. In this manner, the disintegration rate curve is selectively tailorably and distinguishable from mere metal alloys and pure metals that lack the microstructure (i.e., metal matrix and cellular nanomatrix) of the metal composites described herein.

Not only does the microstructure of the metal composite govern the disintegration rate behavior of the metal composite but also affects the strength of the metal composite. As a consequence, the metal composites herein also have a selectively tailorably material strength yield (and other material properties), in which the material strength yield varies due to the processing conditions and the materials used to produce the metal composite. To illustrate, FIG. 7A shows an electron photomicrograph of a fracture surface of a compact formed from a pure Mg powder, and FIG. 7B shows an electron photomicrograph of a fracture surface of an exemplary embodiment of a metal composite with a cellular nanomatrix as described herein. The microstructural morphology of the substantially continuous, cellular nanomatrix, which can be selected to provide a strengthening phase material, with the metal matrix (having particle core material), provides the metal composites herein with enhanced mechanical properties, including compressive strength and sheer strength, since the resulting morphology of the cellular nanomatrix/metal matrix can be manipulated to provide strengthening through the processes that are akin to traditional strengthening mechanisms, such as grain size reduction, solution hardening through the use of impurity atoms, precipitation or age hardening and strain/work hardening mechanisms. The cellular nanomatrix/metal matrix structure tends to limit dislocation movement by virtue of the numerous particle nanomatrix interfaces, as well as interfaces between discrete layers within the cellular nanomatrix material as described herein. This is exemplified in the fracture behavior of these materials, as illustrated in FIGS. 7A and 7B. In FIG. 7A, a compact made using uncoated pure Mg powder and subjected to a shear stress sufficient to induce failure demonstrated intergranular fracture. In contrast, in FIG. 7B, a metal composite made using powder particles having pure Mg powder particle cores to form metal matrix and metallic coating layers that includes Al to form the cellular nanomatrix and subjected to a shear stress sufficient to induce failure demonstrated transgranular fracture and a substantially higher fracture stress as described herein. Because these materials have high-strength characteristics, the core material and coating material may be selected to utilize low density materials or other low density materials, such as low-density metals, ceramics, glasses or carbon, that otherwise would not provide the necessary strength characteristics for use in the desired applications, including well-bore tools and components.

To further illustrate the selectively tailorable material properties of the metal composites having a cellular nanomatrix, FIG. 8 shows a graph of the compressive strength of a metal

composite with a cellular nanomatrix versus weight percentage of a constituent ( $Al_2O_3$ ) of the cellular nanomatrix. FIG. 8 clearly shows the effect of varying the weight percentage (wt %), i.e., thickness, of an alumina coating on the room temperature compressive strength of a metal composite with a cellular nanomatrix formed from coated powder particles that include a multilayer ( $Al/Al_2O_3/Al$ ) metallic coating layer on pure Mg particle cores. In this example, optimal strength is achieved at 4 wt % of alumina, which represents an increase of 21% as compared to that of 0 wt % alumina.

Thus, the metal composites herein can be configured to provide a wide range of selectable and controllable corrosion or disintegration behavior from very low corrosion rates to extremely high corrosion rates, particularly corrosion rates that are both lower and higher than those of powder compacts that do not incorporate the cellular nanomatrix, such as a compact formed from pure Mg powder through the same compaction and sintering processes in comparison to those that include pure Mg dispersed particles in the various cellular nanomaterials described herein. These metal composites 200 may also be configured to provide substantially enhanced properties as compared to compacts formed from pure metal (e.g., pure Mg) particles that do not include the nanoscale coatings described herein. Moreover, metal alloys (formed by, e.g., casting from a melt or formed by metallurgically processing a powder) without the cellular nanomatrix also do not have the selectively tailorable material and chemical properties as the metal composites herein.

As mentioned above, the metal composite is used to produce articles that can be used as tools or implements, e.g., in a downhole environment. In a particular embodiment, the article is a seal, frustoconical member, sleeve, or bottom sub. In another embodiment, combinations of the articles are used together as a disintegrable tubular anchoring system.

Referring to FIGS. 9A and 9B, an embodiment of a disintegrable tubular anchoring system disclosed herein is illustrated at 510. The sealing system 510 includes a frustoconical member 514 (also referred to as a cone and shown individually in FIG. 10) having a first frustoconical portion 516 and a second frustoconical portion 520 that are tapered in opposing longitudinal directions to one another. A bottom sub 570 (shown individually in FIG. 11) is disposed at an end of the disintegrable system 510. Sleeve 524 (shown individually in FIG. 12) is radially expandable in response to being moved longitudinally against the first frustoconical portion 516. Similarly, a seal 528 (shown individually in FIGS. 13A and 13B) is radially expandable in response to being moved longitudinally against the second frustoconical portion 520. One way of moving the sleeve 524 and the seal 528 relative to the frustoconical portions 516, 520 is to compress longitudinally the complete assembly with a setting tool 558. The seal 528 includes a seat 532 with a surface 536 that is tapered in this embodiment and is receptive to a plug 578 that can sealingly engage the surface 536 of seal 528.

The seat 532 of the seal 528 also includes a collar 544 that is positioned between the seal 528 and the second frustoconical portion 520. The collar 544 has a wall 548 whose thickness is tapered due to a radially inwardly facing frustoconical surface 552 thereon. The varied thickness of the wall 548 allows for thinner portions to deform more easily than thicker portions. This can be beneficial for at least two reasons. First, the thinner walled portion 549 can deform when the collar 544 is moved relative to the second frustoconical portion 520 in order for the seal 528 to expand radially into sealing engagement with a structure 540. Second, the thicker walled portion 550 should resist deformation due to pressure differential thereacross that is created when pressuring up against a

plug (e.g., plug 578) seated at the seat 532 during treatment operations, for example. The taper angle of the frustoconical surface 552 may be selected to match a taper angle of the second frustoconical portion 520 thereby to allow the second frustoconical portion 520 to provide radial support to the collar 544 at least in the areas where they are in contact with one another.

The disintegrable tubular anchoring system 510 is configured to set (i.e., anchor) and seal to a structure 540 such as a liner, casing, or closed or open hole in an earth formation borehole, for example, as is employable in hydrocarbon recovery and carbon dioxide sequestration applications. The sealing and anchoring to the structure 540 allows pressure against the plug 578 seated thereat to increase for treatment of the earth formation as is done during fracturing and acid treatment, for example. Additionally, the seat 532 is positioned in the seal 528 such that pressure applied against a plug seated on the seat 532 urges the seal 528 toward the sleeve 524 to thereby increase both sealing engagement of the seal 528 with the structure 540 and the frustoconical member 514 as well as increasing the anchoring engagement of the sleeve 524 with the structure 540.

The sealing system 510 can be configured such that the sleeve 524 is anchored (positionally fixed) to the structure 540 prior to the seal 528 sealingly engaging with the structure 540, or such that the seal 528 is sealingly engaged with the structure 540 prior to the sleeve 524 anchoring to the structure 540. Controlling which of the seal 528 and the sleeve 524 engages with the structure 540 first can be selected through material properties relationships (e.g., relative compressive strength) or dimensional relationships between the components involved in the setting of the seal 528 in comparison to the components involved in the setting of the sleeve 524. Regardless of whether the sleeve 524 or the seal 528 engages the structure 540 first may be set in response to directions of portions of a setting tool that set the disintegrable tubular anchoring system 510. Damage to the seal 528 can be minimized by reducing or eliminating relative movement between the seal 528 and the structure 540 after the seal 528 is engaged with the structure 540. In this embodiment, having the seal 528 engage with the structure 540 prior to having the sleeve 524 engage the structure 540 can achieve this goal.

The surface 536 of the seat 532 is positioned longitudinally upstream (as defined by fluid flow that urges a plug against the seat 532) of the sleeve 524. Additionally, the seat 532 of the seal can be positioned longitudinally upstream of the collar 544 of the seal 528. This relative positioning allows forces generated by pressure against a plug seated against the surface 536 further to urge the seal 528 into sealing engagement with the structure 540.

The portion of the collar 544 that deforms conforms to the second frustoconical portion 520 sufficiently to be radially supported thereby, regardless of whether the taper angles match. The second frustoconical portion 520 can have taper angles from about 1° to about 30°, specifically about 2° to about 20° to facilitate radial expansion of the collar 544 and to allow frictional forces between the collar 544 and the second frustoconical portion 520 to maintain positional relationships therebetween after removal of longitudinal forces that caused the movement therebetween. The first frustoconical portion 516 can also have taper angles from about 10° to about 30°, specifically about 14° to about 20° for the same reasons that the second frustoconical portion 520 does. Either or both of the frustoconical surface 552 and the second frustoconical portion 520 can include more than one taper angle as is illustrated herein on the second frustoconical portion 520 where a nose 556 has a larger taper angle than the surface 520

has further from the nose 556. Having multiple taper angles can provide operators with greater control over amounts of radial expansion of the collar 544 (and subsequently the seal 528) per unit of longitudinal movement between the collar 544 and the frustoconical member 514. The taper angles, in addition to other variables, also provide additional control over longitudinal forces needed to move the collar 544 relative to the frustoconical member 514. Such control can allow the disintegrable tubular anchoring system 510 to expand the collar 544 of the seal 528 to set the seal 528 prior to expanding and setting the sleeve 224.

In an embodiment, the setting tool 558 is disposed along the length of the system 510 from the bottom sub 570 to the seal 528. The setting tool 558 can generate the loads needed to cause movement of the frustoconical member 514 relative to the sleeve 524. The setting tool 558 can have a mandrel 560 with a stop 562 attached to one end 564 by a force failing member 566 such as a plurality of shear screws. The stop 562 is disposed to contact the bottom sub 570. A plate 568 disposed to contact the seal 528 guidingly movable along the mandrel 560 (by means not shown herein) in a direction toward the stop 562 at the bottom sub 570 can longitudinally urge the frustoconical member 514 toward the sleeve 524. Loads to fail the force failing member 566 can be set to only occur after the sleeve 524 has been radially altered by the frustoconical member 514 a selected amount. After failure of the force failing member 566, the stop 562 may separate from the mandrel 560, thereby allowing the mandrel 560 and the plate 568 to be retrieved to surface, for example.

According to an embodiment, the surface 572 of the sleeve 524 includes protrusions 574, which may be referred to as teeth, configured to bitingly engage with a wall 576 of the structure 540, within which the disintegrable system 510 is employable, when the surface 572 is in a radially altered (i.e., expanded) configuration. This biting engagement serves to anchor the disintegrable system 510 to the structure 540 to prevent relative movement therebetween. Although the structure 540 disclosed in this embodiment is a tubular, such as a liner or casing in a borehole, it could be an open hole in an earth formation, for example.

FIG. 9B shows the disintegrable system 510 after the setting tool 558 has been removed from the structure 540 subsequent to setting the disintegrable system 510. Here, the protrusions 574 of the sleeve 524 bitingly engage the wall 576 of the structure 540 to anchor the disintegrable system 510 thereto. Additionally, the seal 528 has been radially expanded to contact the wall 576 of the structure 540 on the outer surface of the seal 528 due to compression thereof by the setting tool 558. The seal 528 deforms such that the length of the seal 528 has increased as the thickness 548 has decreased during compression of the seal 528 between the frustoconical member 514 and the wall 576 of structure 540. In this way, the seal 528 forms a metal-to-metal seal against the frustoconical member 514 and a metal-to-metal seal against the wall 576. Alternatively, the seal 528 can deform to complement topographical features of the wall 576 such as voids, pits, protrusions, and the like. Similarly, the ductility and tensile strength of the seal 528 allow the seal 528 to deform to complement topographical features of the frustoconical member 514.

After setting the disintegrable system 510 with the protrusions 574 of the sleeve 514, a plug 578 can be disposed on the surface 536 of seat 532. Once the plug 578 is sealingly engaged with the seat 532, pressure can increase upstream thereof to perform work such as fracturing an earth formation or actuating a downhole tool, for example, when employed in a hydrocarbon recovery application.

In an embodiment, as shown in FIG. 9B, the plug 578, e.g., a ball, engages the seat 532 of seal 528. Pressure is applied, for example, hydraulically, to the plug 578 to deform the collar 544 of the seal 528. Deformation of the collar 544 causes the wall material 548 to elongate and sealably engage with the structure 540 (e.g., borehole casing) to form a metal-to-metal seal with the first frustoconical portion 516 of the frustoconical member 514 and to form another metal-to-metal seal with the structure 576. Here, the ductility of the metal composite allows the seal 528 to fill the space between the structure 540 and the frustoconical member 514. A down-hole operation can be performed at this time, and the plug 578 subsequently removed after the operation. Removal of the plug 578 from the seat 532 can occur by creating a pressure differential across the plug 578 such that the plug 578 dislodges from the seat 532 and moves away from the seal 528 and frustoconical member 514. Thereafter, any of the seal 528, frustoconical member 514, sleeve 524, or bottom sub 570 can be disintegrated by contact with a downhole fluid. Alternatively, before the plug 578 is removed from the seat 532, a downhole fluid can contact and disintegrate the seal 528, and the plug 578 then can be removed from any of the remaining components of the disintegrable system 510. Disintegration of the seal 528, frustoconical member 514, sleeve 524, or bottom sub 570 is beneficial at least in part because the flow path of the borehole is restored without mechanically removing the components of the disintegrable system 510 (e.g., by boring or milling) or flushing the debris out of the borehole. It should be appreciated that the disintegration rates of the components of the disintegrable system 510 are independently selectively tailorable as discussed above, and that the seal 528, frustoconical member 514, sleeve 524, or bottom sub 570 have independently selectively tailorable material properties such as yield strength and compressive strength.

According to another embodiment, the disintegrable tubular anchoring system 510 is configured to leave a through bore 580 with an inner radial dimension 582 and outer radial dimension 584 defined by a largest radial dimension of the disintegrable system 510 when set within the structure 540. In an embodiment, the inner radial dimension 582 can be large enough for mandrel 560 of the setting tool 558 to fit through the system 510. The stop 562 of the setting tool 558 can be left in the structure 540 after setting the disintegrable system 510 and removal of the mandrel 560. The stop 562 can be fished out of the structure 540 after disintegrating the system 510 at least to a point where the stop 562 can pass through the inner radial dimension 582. Thus, a component of the disintegrable system 510 can be substantially solid. By incorporation of the through bore 580 in the disintegrable system 510, a fluid can be circulated through the disintegrable system 510 from either the downstream or upstream direction in the structure 540 to cause disintegration of a component (e.g., the sleeve).

In another embodiment, the disintegrable tubular anchoring system 510 is configured with the inner radial dimension 582 that is large in relation to the outer radial dimension 584. According to one embodiment, the inner radial dimension 582 is greater than 50% of the outer radial dimension 584, specifically greater than 60%, and more specifically greater than 70%.

The seal, frustoconical member, sleeve, and bottom sub can have beneficial properties for use in, for example a down-hole environment, either in combination or separately. These components are disintegrable and can be part of a completely disintegrable anchoring system herein. Further, the components have mechanical and chemical properties of the metal composite described herein. The components thus beneficially are selectively and tailorably disintegrable in response

to contact with a fluid or change in condition (e.g., pH, temperature, pressure, time, and the like). Exemplary fluids include brine, mineral acid, organic acid, or a combination comprising at least one of the foregoing.

A cross sectional view of an embodiment of a frustoconical member is shown in FIG. 10. As described above, the frustoconical member 514 has a first frustoconical portion 516, second frustoconical portion 520, and nose 556. The taper angle of the frustoconical member 514 can vary along the outer surface 584 so that the frustoconical member 514 has various cross sectional shapes including the truncated double cone shape shown. The wall thickness 586 therefore can vary along the length of the frustoconical member 514, and the inner diameter of the frustoconical member 514 can be selected based on a particular application. The frustoconical member 514 can be used in various applications such as in the disintegrable tubular anchoring system herein as well as in any situation in which a strong or disintegrable frustoconical shape is useful. Exemplary applications include a bearing, flare fitting, valve stem, sealing ring, and the like.

A cross sectional view of a bottom sub is shown in FIG. 11. The bottom sub 700 has a first end 702, second end 704, optional thread 706, optional through holes 708, inner diameter 710, and outer diameter 712. In an embodiment, the bottom sub 700 is the terminus of a tool (e.g., disintegrable system 510). In another embodiment, the bottom sub 700 is disposed at an end of a string. In certain embodiment, the bottom sub 700 is used to attach tools to a string. Alternatively, the bottom sub 700 can be used between tools or strings and can be part of a joint or coupling. The bottom sub 700 can be used with a string and an article such as a bridge plug, frac plug, mud motor, packer, whip stock, and the like. In one non-limiting embodiment, the first end 702 provides an interface with, e.g., the frustoconical member 514 and the sleeve 524. The second end 704 engages the stop 562 of the setting tool 558. Thread 706, when present, can be used to secure the bottom sub 700 to an article. In an embodiment, the frustoconical member 514 has a threaded portion that mates with the thread 706. In some embodiments, thread 706 is absent, and the inner diameter 710 can be a straight bore or can have portions thereof that are tapered. The through holes 708 can transmit fluid, e.g., brine, to disintegrate the bottom sub 700 or other components of the disintegrable system 510. The through holes also can be an attachment point for the force failing member 566 used in conjunction with the setting tool 558 or similar device. It is contemplated that the bottom sub 700 can have another cross sectional shape than that shown in FIG. 11. Exemplary shapes include a cone, ellipsoid, toroid, sphere, cylinder, their truncated shapes, asymmetrical shapes, including a combination of the foregoing, and the like. Further, the bottom sub 700 can be a solid item or can have an inner diameter that is at least 10% the size of the outer diameter, specifically at least 50%, and more specifically at least 70%.

A sleeve is shown in a perspective, cross sectional, and top views respectively in FIGS. 12A, 12B, and 12C. The sleeve 524 includes an outer surface 572, protrusions 574 disposed on the outer surface 572, and inner surface 571. The sleeve 524 acts as a slip ring with the protrusions 574 as slips that bitingly engage a surface such as a wall of a casing or open hole as the sleeve 524 radially expands in response to a first portion 573 of the inner surface 571 engaging a mating surface (e.g., first frustoconical portion 516 in FIG. 10). The protrusions 574 can circumferentially surround the entirety of the sleeve 524. Alternatively, the protrusions 574 can be spaced apart, either symmetrically or asymmetrically, as shown in the top view in FIG. 12C. The shape of the sleeve

524 is not limited to that shown in FIG. 12. The sleeve, in addition to being a slip ring in the disintegrable tubular anchoring system illustrated in FIG. 9, can be used to set numerous tools including a packer, bridge plug, or frac plug or can be disposed in any environment where anti-slipping of an article can be accomplished by engaging the protrusions of the sleeve with a mating surface.

Referring to FIGS. 13A and 13B, a seal 400 includes an inner sealing surface 402, outer sealing surface 404, seat 406, and a surface 408 of the seat 406. The surface 408 is configured (e.g., shaped) to accept a member (e.g., a plug) to provide force on the seal 400 in order to deform the seal so that the inner sealing surface 402 and outer sealing surface 404 respectively form metal-to-metal seals with mating surfaces (not shown in FIGS. 13A and 13B). Alternatively, a compressive force is applied to the seal 400 by a frustoconical member and setting tool disposed at opposing ends of the seal 400 as in FIG. 9A. In an embodiment, the seal 400 is useful in a downhole environment as a conformable, deformable, highly 10 ductile, and disintegrable seal. In an embodiment, the seal 400 is a bridge plug, gasket, flapper valve, and the like.

In addition to being selectively corrodible, the seal herein deforms in situ to conform to a space in which it is disposed in response to an applied setting pressure, which is a pressure 25 large enough to expand radially the seal or to decrease the wall thickness of the seal by increasing the length of the seal. Unlike many seals, e.g., an elastomer seal, the seal herein is prepared in a shape that corresponds to a mating surface to be sealed, e.g., a casing, or frustoconical shape of a downhole 30 tool. In an embodiment, the seal is a temporary seal and has an initial shape that can be run downhole and subsequently deformed under pressure to form a metal-to-metal seal that deforms to surfaces that the seal contacts and fills spaces (e.g. voids) in a mating surface. To achieve the sealing properties, 35 the seal has a percent elongation of about 10% to about 75%, specifically about 15% to about 50%, and more specifically about 15% to about 25%, based on the original size of the seal. The seal has a yield strength of about 15 kilopounds per square inch (ksi) to about 50 ksi, and specifically about 15 ksi 40 to about 45 ksi. The compressive strength of the seal is from about 30 ksi to about 100 ksi, and specifically about 40 ksi to about 80 ksi. To deform the seal, a pressure of up to about 10,000 psi, and specifically about 9,000 psi can be applied to the seal.

45 Unlike elastomeric seals, the seal herein that includes the metal composite has a temperature rating up to about 1200° F., specifically up to about 1000° F., and more specifically up to about 800° F. The seal is temporary in that the seal is selectively and tailorably disintegrable in response to contact with a downhole fluid or change in condition (e.g., pH, temperature, pressure, time, and the like). Exemplary downhole 50 fluids include brine, mineral acid, organic acid, or a combination comprising at least one of the foregoing.

55 Since the seal interworks with other components, e.g., a frustoconical member, sleeve, or bottom sub in, e.g., the disintegrable tubular anchoring system herein, the properties of each component are selected for the appropriate relative selectively tailorable material and chemical properties. These properties are a characteristic of the metal composite and the 60 processing conditions that form the metal composite, which is used to produce such articles, i.e., the components. Therefore, in an embodiment, the metal composite of a component will differ from that of another component of the disintegrable system. In this way, the components have independent selectively tailorable mechanical and chemical properties.

65 According to an embodiment, the sleeve and seal deform under a force imparted by the frustoconical member and

bottom sub. To achieve this result, the sleeve and seal have a compressive strength that is less than that of the bottom sub or frustoconical member. In another embodiment, the sleeve deforms before, after, or simultaneously as deformation of the seal. It is contemplated that the bottom sub or frustoconical member deforms in certain embodiments. In an embodiment, a component has a different amount of a strengthening agent than another component, for example, where a higher strength component has a greater amount of strengthening agent than does a component of lesser strength. In a specific embodiment, the frustoconical member has a greater amount of strengthening agent than that of the seal. In another embodiment, the frustoconical member has a greater amount of strengthening agent than that of the sleeve. Similarly, the bottom sub can have a greater amount of strengthening agent than either the seal or sleeve. In a particular embodiment, the frustoconical member has a compressive strength that is greater than that of either the seal or sleeve. In a further embodiment, the frustoconical member has a compressive strength that is greater than that of either of the seal or sleeve. In one embodiment, the frustoconical member has a compressive strength of 40 ksi to 100 ksi, specifically 50 ksi to 100 ksi. In another embodiment, the bottom sub has a compressive strength of 40 ksi to 100 ksi, specifically 50 ksi to 100 ksi. In yet another embodiment, the seal has a compressive strength of 30 ksi to 70 ksi, specifically 30 ksi to 60 ksi. In yet another embodiment, the sleeve has a compressive strength of 30 ksi to 80 ksi, specifically 30 ksi to 70 ksi. Thus, under a compressive force either the seal or sleeve will deform before deformation of either the bottom sub or frustoconical member.

Other factors that can affect the relative strength of the components include the type and size of the strengthening agent in each component. In an embodiment, the frustoconical member includes a strengthening of smaller size than a strengthening agent in either of the seal or sleeve. In yet another embodiment, the bottom sub includes a strengthening agent of smaller size than a strengthening agent in either of the seal or sleeve. In one embodiment, the frustoconical member includes a strengthening agent such as a ceramic, metal, cermet, or a combination thereof, wherein the size of the strengthening agent is from 10 nm to 200  $\mu$ m, specifically 100 nm to 100  $\mu$ m.

Yet another factor that impacts the relative selectively tailorable material and chemical properties of the components is the constituents of the metal composite, i.e., the metallic nanomatrix of the cellular nanomatrix, the metal matrix disposed in the cellular nanomatrix, or the disintegration agent. The compressive and tensile strengths and disintegration rate are determined by the chemical identity and relative amount of these constituents. Thus, these properties can be regulated by the constituents of the metal composite. According to an embodiment, a component (e.g., seal, frustoconical member, sleeve, or bottom sub) has a metal matrix of the metal composite that includes a pure metal, and another component has a metal matrix that includes an alloy. In another embodiment, the seal has a metal matrix that includes a pure metal, and the frustoconical member has a metal matrix that includes an alloy. In an additional embodiment, the sleeve has a metal matrix that is a pure metal. It is contemplated that a component can be functionally graded in that the metal matrix of the metal composite can contain both a pure metal and an alloy having a gradient in the relative amount of either the pure metal or alloy in the metal matrix as disposed in the component. Therefore, the value of the selectively tailorable properties varies in relation to the position along the component.

In a particular embodiment, the disintegration rate of a component (e.g., seal, frustoconical member, sleeve, or bot-

tom sub) has a greater value than that of another component. Alternatively, each component can have substantially the same disintegration rate. In a further embodiment, the sleeve has a greater disintegration rate than another component, e.g., the frustoconical member. In another embodiment, the amount of disintegration agent of a component (e.g., seal, frustoconical member, sleeve, or bottom sub) is present in an amount greater than that of another component. In another embodiment, the amount of disintegration agent present in the sleeve is greater than another component. In one embodiment, the amount of disintegrating agent in the seal is greater than another component.

Referring to FIGS. 14 and 15, an alternate embodiment of a disintegrable tubular anchoring system is illustrated at 1110. The disintegrable system 1110 includes a frustoconical member 1114, a sleeve 1118 having a surface 1122, a seal 1126 having a surface 1130, and a seat 1134, wherein each component is made of the metal composite and has selectively tailorable mechanical and chemical properties herein. A primary difference between the system 510 (FIG. 9) and the system 1110 is the initial relative position of the seal and frustoconical member.

An amount of radial alteration that the surface 1122 of the sleeve 1118 undergoes is controlled by how far the frustoconical member 1114 is forced into the sleeve 1118. A frustoconical surface 1144 on the frustoconical member 1114 is wedgably engagable with a frustoconical surface 1148 on the sleeve 1118. As such, the further the frustoconical member 1114 is moved relative to the sleeve 1118, the greater the radial alteration of the sleeve 1118. Similarly, the seal 1126 is positioned radially of the frustoconical surface 1144 and is longitudinally fixed relative to the sleeve 1118 so the further the frustoconical member 1114 moves relative to the sleeve 1118 and the seal 1126, the greater the radial alteration of the seal 1126 and the surface 1130. The foregoing structure allows an operator to determine the amount of radial alteration of the surfaces 1122, 1130 after the system 1110 is positioned within a structure 1150.

Optionally, the system 1110 can include a collar 1154 positioned radially between the seal 1126 and the frustoconical member 1114 such that a radial dimension of the collar 1154 is also altered by the frustoconical member 1114 in response to the movement relative thereto. The collar 1154 can have a frustoconical surface 1158 complementary to the frustoconical surface 1144 such that substantially the full longitudinal extent of the collar 1154 is simultaneously radially altered upon movement of the frustoconical member 1114. The collar 1154 may be made of a metal composite that is different than that of the seal 1126 or that of the frustoconical member 1114. Thus, collar 1154 can maintain the seal 1126 at an altered radial dimension even if the frustoconical surface 1144 is later moved out of engagement with the frustoconical surface 1158, thereby maintaining the seal 1126 in sealing engagement with a wall 1162 of the structure 1150. This can be achieved by selecting the metal composite of the collar 1154 to have a higher compressive strength than that of the seal 1126.

The disintegrable system 1110 further includes a land 1136 on the frustoconical member 1114 sealably engagable with the plug 1138. Also included in the disintegrable system are a recess 1166 (within a wall 1058) of the sleeve 1118 receptive to shoulders 1170 on fingers 1174, which provisions are engagable together once the setting tool 558 compresses the disintegrable system 1110 in a similar manner as the disintegrable system 510 is settable with the setting tool 558 as shown in FIG. 9.

Referring to FIG. 16, another alternate embodiment of a disintegrable tubular anchoring system is illustrated at 1310. The disintegrable system 1310 includes a first frustoconical member 1314, sleeve 1318 positioned and configured to be radially expanded into anchoring engagement with a structure 1322, illustrated herein as a wellbore in an earth formation 1326, in response to being urged against a frustoconical surface 1330 of the first frustoconical member 1314. A collar 1334 is radially expandable into sealing engagement with the structure 1322 in response to being urged longitudinally relative to a second frustoconical member 1338 and has a seat 1342 with a surface 1346 sealingly receptive to a plug 1350 (shown with dashed lines) runnable thereagainst. The seat 1342 is displaced in a downstream direction (rightward in FIG. 16) from the collar 1334 as defined by fluid that urges the plug 1350 against the seat 1342. This configuration and position of the surface 1346 relative to the collar 1334 aids in maintaining the collar 1334 in a radially expanded configuration (after having been expanded) by minimizing radial forces on the collar 1334 due to pressure differential across the seat 1342 when plugged by a plug 1350.

To clarify, if the surface 1346 were positioned in a direction upstream of even a portion of the longitudinal extend of the collar 1334 (which it is not) then pressure built across the plug 1350 seated against the surface 1346 would generate a pressure differential radially across the portion of the collar 1334 positioned in a direction downstream of the surface 1346. This pressure differential would be defined by a greater pressure radially outwardly of the collar 1334 than radially inwardly of the collar 1334, thereby creating radially inwardly forces on the collar 1334. These radially inwardly forces, if large enough, could cause the collar 1334 to deform radially inwardly potentially compromising the sealing integrity between the collar 1334 and the structure 1322 in the process. This condition is specifically avoided by the positioning of the surface 1346 relative to the collar 1334.

Optionally, the disintegrable tubular anchoring system 1310 includes a seal 1354 positioned radially of the collar 1334 configured to facilitate sealing of the collar 1334 to the structure 1322 by being compressed radially therebetween when the collar 1334 is radially expanded. The seal 1354 is fabricated from a metal composite that has a lower compressive strength than that of the first frustoconical member 1314 to enhance sealing of the seal 1354 to both the collar 1334 and the structure 1322. In an embodiment, the seal 1354 has a lower compressive strength than that of the collar 1334.

Thus in this embodiment, the disintegrable system 1310 can include a first frustoconical member 1314, sleeve 1318, and an optional seal 1354. In the instance when the seal 1354 is not present, the collar 1334 of the first frustoconical member 1314 can form a metal-to-metal seal with the casing or liner or conform to an openhole surface. In some embodiments, the first frustoconical member 1314 contains a functionally graded metal composite such that the collar 1334 has a lower compressive strength value than that of the rest of the first frustoconical member 1314. In another embodiment the collar 1334 has a lower compressive strength than that of the second frustoconical member 1338. In yet another embodiment, the second frustoconical member 1338 has a greater compressive strength than that of the seal 1354.

The components herein can be augmented with various materials. In one embodiment, a seal, e.g., seal 528, can include a backup seal such as an elastomer material 602 as shown in FIG. 17. The elastomer can be, for example, an O-ring disposed in a gland 604 on the surface of the seal 528. The elastomer material includes but not limited to, for example, butadiene rubber (BR), butyl rubber (IIR), chloro-

sulfonated polyethylene (CSM), epichlorohydrin rubber (ECH, ECO), ethylene propylene diene monomer (EPDM), ethylene propylene rubber (EPR), fluoroelastomer (FKM), nitrile rubber (NBR, HNBR, HSN), perfluoroelastomer (FFKM), polyacrylate rubber (ACM), polychloroprene (neoprene) (CR), polyisoprene (IR), polysulfide rubber (PSR), sanifluor, silicone rubber (SiR), styrene butadiene rubber (SBR), or a combination comprising at least one of the foregoing.

10 As described herein, the components, e.g., the seal, can be used in a downhole environment, for example, to provide a metal-to-metal seal. In an embodiment, a method for temporarily sealing a downhole element includes disposing a component downhole and applying pressure to deform the component. The component can include a seal, frustoconical member, sleeve, bottom, or a combination comprising at least one of the foregoing. The method also includes conforming the seal to a space to form a temporary seal, compressing the sleeve to engage a surface, and thereafter contacting the component with a downhole fluid to disintegrate the component. The component includes the metal composite herein having a metal matrix, disintegration agent, cellular nanomatrix, and optionally strengthening agent. The metal composite of the seal forms an inner sealing surface and an outer sealing surface disposed radially from the inner sealing surface of the seal.

According to an embodiment, a process of isolating a structure includes disposing a disintegrable tubular anchoring system herein in a structure (e.g., tubular, pipe, tube, borehole 30 (closed or open), and the like), radially altering the sleeve to engage a surface of the structure, and radially altering the seal to the isolate the structure. The disintegrable tubular anchoring system can be contacted with a fluid to disintegrate, e.g., the seal, frustoconical member, sleeve, bottom sub or a combination of at least one of the foregoing. The process further can include setting the disintegrable anchoring system with a setting tool. Additionally, a plug can be disposed on the seal. Isolating the structure can be completely or substantially impeding fluid flow through the structure.

40 Moreover, the seal can have various shapes and sealing surfaces besides the particular arrangement shown in FIGS. 9 and 13-16. In another embodiment, Referring to FIGS. 18A and 18B, an embodiment of a seal disclosed herein is illustrated at 100. The seal 100 includes a metal composite, a first sealing surface 102, and a second sealing surface 104 opposingly disposed from the first sealing surface 102. The metal composite includes a metal matrix disposed in a cellular nanomatrix, a disintegration agent, and optionally a strengthening agent. The seal 100 can be any shape and conforms in situ under pressure to a surface to form a temporary seal that is selectively disintegrable in response to contact with a fluid. In this embodiment, the seal 100 is an annular shape with an outer diameter 106 and inner diameter 108. In some embodiments, the first surface 102, second surface 104, outer diameter 106, inner diameter 108, or a combination comprising at 50 55 least one of the foregoing can be a sealing surface.

Although variations of a disintegrable tubular anchoring system have described that include several components together, it is contemplated that each component is separately 60 and independently applicable as an article. Further, any combination of the components can be used together. Moreover, the components can be used in surface or downhole environments.

While one or more embodiments have been shown and 65 described, modifications and substitutions may be made thereto without departing from the spirit and scope of the invention. Accordingly, it is to be understood that the present

invention has been described by way of illustrations and not limitation. Embodiments herein are can be used independently or can be combined.

All ranges disclosed herein are inclusive of the endpoints, and the endpoints are independently combinable with each other. The suffix "(s)" as used herein is intended to include both the singular and the plural of the term that it modifies, thereby including at least one of that term (e.g., the colorant (s) includes at least one colorants). "Optional" or "optionally" means that the subsequently described event or circumstance can or cannot occur, and that the description includes instances where the event occurs and instances where it does not. As used herein, "combination" is inclusive of blends, mixtures, alloys, reaction products, and the like. All references are incorporated herein by reference.

The use of the terms "a" and "an" and "the" and similar referents in the context of describing the invention (especially in the context of the following claims) are to be construed to cover both the singular and the plural, unless otherwise indicated herein or clearly contradicted by context. As used herein, the term "a" includes at least one of an element that "a" precedes, for example, "a device" includes "at least one device." "Or" means "and/or." Further, it should further be noted that the terms "first," "second," and the like herein do not denote any order, quantity (such that more than one, two, or more than two of an element can be present), or importance, but rather are used to distinguish one element from another. The modifier "about" used in connection with a quantity is inclusive of the stated value and has the meaning dictated by the context (e.g., it includes the degree of error associated with measurement of the particular quantity).

What is claimed is:

1. A frustoconical member comprising:  
a metal composite which includes:  
a cellular nanomatrix comprising a metallic nanomatrix material; and  
a metal matrix disposed in the cellular nanomatrix,  
wherein the frustoconical member comprises a first frustoconical portion; and  
wherein the frustoconical member has a disintegration rate of about 1 mg/cm<sup>2</sup>/hr to about 10,000 mg/cm<sup>2</sup>/hr.
2. The frustoconical member of claim 1, further comprising a second frustoconical portion.
3. The frustoconical member of claim 2, wherein the first frustoconical portion and second frustoconical portion are tapered in opposing directions to one another.
4. The frustoconical member of claim 1, further comprising an inner radial dimension and outer radial dimension such that the inner radial dimension is greater than 50% of the outer radial dimension.
5. The frustoconical member of claim 1, further comprising a seat disposed at an inner surface of the frustoconical member.
6. The frustoconical member of claim 1, wherein the metal matrix comprises aluminum, iron, magnesium, manganese, zinc, or a combination comprising at least one of the foregoing.
7. The frustoconical member of claim 1, wherein the amount of the metal matrix is about 50 wt % to about 95 wt %, based on the weight of the metal composite.
8. The frustoconical member of claim 1, wherein the metal matrix is an alloy, pure metal, or a combination comprising at least one of the foregoing.
9. The frustoconical member of claim 8, wherein the frustoconical member is functionally graded such that the metal

matrix includes an alloy or a pure metal, wherein the amount of the alloy or pure metal varies along a dimension of the frustoconical member.

10. The frustoconical member of claim 1, wherein the metallic nanomatrix material comprises aluminum, cobalt, copper, iron, magnesium, nickel, silicon, tungsten, zinc, an oxide thereof, a nitride thereof, a carbide thereof, an intermetallic compound thereof, a cermet thereof, or a combination comprising at least one of the foregoing.
11. The frustoconical member of claim 1, wherein the amount of the metal nanomatrix material is about 10 wt % to about 50 wt %, based on the weight of the metal composite.
12. The frustoconical member of claim 1, wherein the metal composite further includes a strengthening agent.
13. The frustoconical member of claim 12, wherein the strengthening agent comprises a ceramic, polymer, metal, nanoparticles, cermet, or a combination comprising at least one of the foregoing.
14. The frustoconical member of claim 12, wherein the frustoconical member is functionally graded such that an amount of the strengthening agent in the first frustoconical portion is greater than an amount of the strengthening agent in another portion of the frustoconical member.
15. The frustoconical member of claim 1, wherein the frustoconical member is functionally graded such that the first frustoconical portion has a compressive strength which is greater than a compressive strength in another portion of the frustoconical member.
16. The frustoconical member of claim 1, wherein the frustoconical member is disintegrable in response to contact with a fluid.
17. The frustoconical member of claim 1, wherein the fluid comprises brine, mineral acid, organic acid, or a combination comprising at least one of the foregoing.
18. An article comprising the frustoconical member of claim 1, wherein the article is a frac plug, bridge plug, bearing, flare fitting, valve stem, or sealing ring.
19. A frustoconical member comprising:  
a metal composite which includes:  
a cellular nanomatrix comprising a metallic nanomatrix material; and  
a metal matrix disposed in the cellular nanomatrix;  
wherein the frustoconical member comprises:  
a first frustoconical portion; and  
a seat disposed at an inner surface of the frustoconical member; and  
wherein the seat includes a land which is sealingly engagable with a removable plug runnable thereagainst, the land being longitudinally disposed relative to the first frustoconical portion in an upstream direction defined by direction of flow that urges the plug thereagainst.
20. The frustoconical member of claim 19, further comprising a collar disposed radially from the land.
21. The frustoconical member of claim 20, herein the collar has a compressive strength which is less than that of the first frustoconical portion.
22. A frustoconical member comprising:  
a metal composite which includes:  
a cellular nanomatrix comprising a metallic nanomatrix material; and  
a metal matrix disposed in the cellular nanomatrix;  
wherein the frustoconical member comprises:  
a first frustoconical portion; and  
wherein the metal composite further comprises a disintegration agent.

**25**

**23.** The frustoconical member of claim **22** wherein the disintegration agent comprises cobalt, copper, iron, nickel, tungsten, or a combination comprising at least one of the foregoing.

**24.** The frustoconical member of claim **22**, wherein the frustoconical member is functionally graded such that an amount of the disintegration agent in the first frustoconical portion is less than an amount of the disintegration agent in another portion of the frustoconical member.

**25.** A frustoconical member comprising:

a metal composite which includes:

    a cellular nanomatrix comprising a metallic nanomatrix material; and

    a metal matrix disposed in the cellular nanomatrix; wherein the frustoconical member comprises:

    a first frustoconical portion; and

    wherein the frustoconical member has a compressive strength of about 40 ksi to about 100 ksi.

**26.** A process of making a frustoconical member of claim **1**, the process comprising:

    combining a metal matrix powder, a disintegration agent, and metal nanomatrix material to form a composition; compacting the composition to form a compacted composition;

    sintering the compacted composition; and

    pressing the sintered composition to form the frustoconical member having a tapered portion on an outer surface of the frustoconical member.

**27.** The process of claim **26**, further comprising disposing a strengthening agent in the composition before compacting the composition.

**28.** A method of using a frustoconical member of claim **1**, the method comprising:

    contacting a frustoconical portion of the frustoconical member to a tapered surface of an article;

**26**

    applying pressure to the frustoconical member; urging the frustoconical member in a direction relative to the article to expand a radial dimension of the article; and

    contacting the frustoconical member with a fluid to disintegrate the frustoconical member.

**29.** A frustoconical member comprising:

a metal composite which includes:

    a cellular nanomatrix comprising a metallic nanomatrix material; and

    a metal matrix disposed in the cellular nanomatrix;

wherein the frustoconical member comprises:

    a first frustoconical portion; and

    wherein the frustoconical member is functionally graded.

**30.** The frustoconical member of claim **29**, wherein:

    the frustoconical member is functionally graded such that the metal matrix includes an alloy or a pure metal, wherein the amount of the alloy or pure metal varies along a dimension of the frustoconical member; or

    the frustoconical member is functionally graded such that an amount of an disintegration agent in the first frustoconical portion is less than an amount of the disintegration agent in another portion of the frustoconical member; or

    the frustoconical member is functionally graded such that an amount of an strengthening agent in the first frustoconical portion is greater than an amount of the strengthening agent in another portion of the frustoconical member; or

    the frustoconical member is functionally graded such that the first frustoconical portion has a compressive strength which is greater than a compressive strength in another portion of the frustoconical member.

\* \* \* \* \*